

July 14, 1936.

W. B. WINES

2,047,349

METHOD OF MANUFACTURING ELECTROSTATIC CONDENSERS

Filed Oct. 20, 1933



FIG. 1



FIG. 2

INVENTOR  
W. B. WINES

BY H. A. Whitehorn

ATTORNEY

## UNITED STATES PATENT OFFICE

2,047,349

METHOD OF MANUFACTURING ELECTRO-  
STATIC CONDENSERSWilliam B. Wines, Elmhurst, Ill., assignor to  
Western Electric Company, Incorporated, New  
York, N. Y., a corporation of New York

Application October 20, 1933, Serial No. 694,505

14 Claims. (Cl. 175—41)

This invention relates to a method of manufacturing electrostatic condensers, and is an improvement in the method of manufacturing condensers of the paper and foil rolled type disclosed in copending application of R. E. Carlson, Serial No. 417,615, filed December 31, 1929, allowed August 21, 1933 and now Patent No. 1,948,331, February 20, 1934.

In the above mentioned application a method of manufacturing condensers of the referred to type is disclosed which includes the step of applying a preliminary pressure to the rolled condensers prior to the baking or dehydrating and impregnating steps, thereafter dehydrating and impregnating the condensers, cooling the condensers to a predetermined temperature without substantial pressure, and then applying pressure until the condensers are completely cooled. This step of applying a preliminary pressure to the condensers prior to the dehydrating and impregnating steps, coupled with the final pressure, resulted in the capacity of the condensers being increased approximately 18% over prior methods wherein no preliminary pressure was applied to the condensers.

The object of this invention is to increase the capacity for a given size and weight of material of the above and similar types of condensers.

In accordance with one method of carrying out the present invention the steps of the method above described are substantially utilized but the method is modified by subjecting the condensers after the baking or dehydrating step and prior to being impregnated to a second pressure followed by a supplementary baking while the latter pressure is applied. By practicing the described method of the present invention there results a further appreciable increase in the capacity of the condensers over that of the condensers manufactured in accordance with the method of the referred to application.

The invention will be more fully understood from the following description, taken in connection with the accompanying drawing, wherein

Fig. 1 is a longitudinal vertical sectional view of a pressing apparatus used in practicing the method, and

Fig. 2 is an enlarged fragmentary plan view of the pressing apparatus shown in Fig. 1.

A pressing apparatus used in practicing the method will be described first and more complete details of the method will follow.

The apparatus for preliminarily pressing the condensers as disclosed in the drawing comprises a compressor 10 which is mounted on a suitable

frame 11, the compressor consisting of a cylinder 12 closed at its ends by end plates 13 and 14. A two-way piston 15 is movably disposed in the cylinder 12 and is provided with a plunger rod 16 which extends through the end plate 13 and a packing gland which is carried thereby. A plunger head 17 is mounted on the outer end of the plunger rod 16 for a purpose hereinafter described. Air lines or pipes 18 and 19 each have one of their ends disposed in communication with the cylinder 12 through the end plates 13 and 14, respectively, while the other ends of the air lines or pipes 18 and 19 are connected to a valve 20 which may be termed as a four-way valve. An air supply line 21 is in communication with the valve 20 and is arranged to supply air under pressure to the cylinder. The valve 20 is provided with arcuate shaped passageways 22 and 23 which are arranged to connect the air lines 18 and 19 with the supply pipe 21 or to connect the air lines 18 and 19 with an exhaust opening 24. A pressure gauge 25 is in communication with the air supply line 21 through a pipe 26 for indicating the pressure of the air in the cylinder 12.

The frame 11 is provided with substantially U-shaped supporting members 28 which are adapted to support a rack 29, and an abutting member 30 against which one end of the rack is disposed. The rack 29 is provided with a bottom portion 31 for supporting a plurality of condensers 32 and their spacing plates 33, and side members 34 for holding the condensers and plates against lateral displacement.

When producing the condensers 32 in accordance with this invention they are wound in the usual manner and placed by the operator within the rack 29, with their ends resting upon the bottom portion 31. The condensers are arranged in layers within the rack 29 and two nickel-silver plates 33 are disposed between each layer. The rack 29 with the condensers and the separating plates 33 is then disposed upon the frame 11 with one end adjacent the abutting member 30 and the other end disposed so that the plunger head 17 may enter an opening 35 within the rack. While in this position the valve 20 is actuated by a handle 36 which is moved from the dotted line position into the full line position shown in Fig. 1. This movement of the valve 20 will allow the air under pressure to pass from the supply pipe 21 through the arcuate shaped passageway 23, the air line 19, and into the cylinder 12, thus forcing the piston 15 toward the end plate 13 and forcing the plunger into the frame 11 through the opening 35 and against the contents thereof.

- While the valve 20 is in this position the air upon the opposite side of the piston 15 will be allowed to escape through the air line 18, the passageway 22, and the exhaust opening 24. The condensers 5 are subjected in this manner to a pressure which is not sufficient to weaken the dielectric strength or specifically to a pressure of approximately 300 pounds resulting in a pressure of approximately 60 pounds per square inch on the sides of each unit or condenser which has approximately 10 square inches of surface. It should be understood, however, that the amount of pressure may vary with the type of condenser employed, and also that a much higher pressure 15 than that mentioned has been employed, for instance, a pressure of approximately eighty pounds per square inch on the sides of the condensers, with good results. In some types of condensers, such as, for instance, the non-inductance type 20 in which terminals are not inserted between the paper and foil, considerably higher pressures may be used, since in such condensers there is no tendency for the terminals to disrupt the paper and foil at the high pressure.
- 25 After the desired amount of pressure has been applied to the condensers 32, wedges such as those indicated at 37 are disposed between the end of the rack 29 and the condensers so as to retain the pressure. The plunger 17 is then removed from the rack 29 by moving the handle 36 into the dotted line position and actuating the valve 20 so as to allow the piston 15 to return to its normal position. The rack 29 of condensers 32 is then removed from the frame 11 and placed in a carrier which is transferred to a treating or impregnating tank (not shown), which consists of chambers internally heated by means of steam plates. The condensers are baked under atmospheric pressure for at least two hours at a temperature of 200° F. to 265° F., then under an absolute pressure of from 2 to 3 inches of mercury at approximately the same temperature for at least four hours, and thereafter under an absolute pressure of not more than 1/2 inch of mercury of the same temperature for at least one hour to thoroughly dehydrate them.
- During the baking of the condensers 32 to dehydrate them the preliminary pressure may be entirely relieved or substantially so due to the 50 shrinkage of the paper or other dielectric material used in the condensers. In order to take up this shrinkage the condensers are subjected to a second pressure immediately after the baking thereof before any appreciable degree of cooling 55 takes place. The pressing apparatus 10 may be used to subject the condensers to the second pressure and in a manner similar to the operation thereof hereinbefore described in connection with the application of the preliminary pressure to the condensers. Therefore, immediately after the baking operation the rack 29 of condensers is transferred again to the pressing apparatus 10 and subjected to a second pressure, the wedges 37 being removed during the application of the pressure. The amount of pressure applied to the condensers during the second pressing operation 60 may be identical to that applied in the preliminary pressing operation, namely, approximately 65 60 pounds per square inch on the sides of each condenser, or it may be of a higher or lower order than the preliminary pressure. This second pressure may be applied to the condensers without stressing the dielectric material any more than 70 75 it was stressed during the preliminary pressure,

which, as hereinbefore described, is not sufficient to weaken the dielectric strength.

After the rack 29 of condensers 32 have been subjected to the desired amount of second pressure the wedges 37 are again disposed between the end of the rack and the condensers so as to retain the pressure and the rack of condensers is again placed in the impregnating tank and subjected under a vacuum to a supplementary baking thereof to bring them to the temperature to 10 which they were subjected in the dehydrating operation previously described.

The impregnating tank is then filled with a compound while the vacuum is maintained and the condensers 32 are thus impregnated under 15 an absolute pressure of not more than 1/2 inch mercury for at least two hours with the temperature remaining as stated above. The vacuum is then released from the condensers while remaining in the compound for approximately five minutes under atmospheric pressure and thereafter the compound is discharged from the tanks. After the condensers have drained slightly, they are removed to a hydraulic press wherein they are subjected to pressure sufficient to take up the 25 contraction of the condensers as they cool. In this press the condensers remain without substantial pressure until they cool to approximately 210° F. and thereafter a pressure of approximately 12 pounds per unit is applied, which results in a pressure of approximately 2 pounds per square inch on the sides of each unit, until they are cooled to 205° F., when the 12 pound pressure is raised to approximately 18 pounds and retained at this pressure until the temperature is reduced 30 to 200° F. Again the pressure is increased to 30 pounds per unit and the condensers are allowed to cool under this pressure to 140° F., after which the rack 29 is removed and the condensers are separated.

The application of a preliminary pressure to the condensers, prior to, and while such pressure is applied during the baking or dehydrating step, the latter step followed by a second pressure and a supplemental baking thereof, and thereafter the treating or impregnating step of this method, while such second pressure is applied, coupled with the subsequent application of pressure, which is increased, during the cooling of the condensers, increases the capacity of the condensers an appreciable degree. The increase in the capacity of the condensers, by this method, not only makes it possible for condensers of a desired capacity to be manufactured smaller in size, so as to require less space during use, but reduces the cost of the condensers in view of the fact that less material is required in producing the condensers of the desired capacity. Furthermore with this method of manufacture, condensers may be increased in capacity without increasing the size thereof.

While the invention has been described with reference to a specific embodiment thereof, it is understood that various modifications may be made therein without departing from the spirit and scope of the present invention.

What is claimed is:

1. A method of manufacturing condensers which comprises applying pressure to compress a condenser, heating the compressed condenser to 70 expel moisture and gases, applying pressure to compress the condenser, heating the compressed condenser, impregnating the condenser, cooling the condenser to a predetermined temperature without substantial pressure, and then compress-

ing the condenser under a relatively low pressure until the condenser is completely cooled.

2. A method of manufacturing condensers which comprises preliminarily compressing a condenser, heating the compressed condenser, applying an increasing vacuum to the compressed condenser while heating to expel moisture and gases, again compressing the condenser, heating the condenser, impregnating the compressed condenser, cooling the condenser to a predetermined temperature without substantial compression, and then compressing the condenser during the remainder of the cooling operation, the pressures of the preliminary and second compressions being higher than the final pressure.

3. A method of manufacturing condensers which comprises preliminarily compressing a condenser under a high pressure, heating the compressed condenser, compressing the condenser under a second high pressure, heating the condenser, impregnating the compressed condenser, cooling the condenser to a predetermined temperature, and then compressing the condenser under a relatively low pressure during the remainder of the cooling operation.

4. A method of manufacturing condensers which comprises preliminarily compressing a condenser, baking the compressed condenser, again compressing the condenser, baking the compressed condenser, impregnating the condenser at the residual pressure remaining from the second compression, cooling the condenser, compressing the condenser during the cooling thereof, the preliminary and second pressures for compressing the condenser being higher than the final pressure.

5. A method of manufacturing condensers which comprises preliminarily compressing a condenser under a pressure in the vicinity of sixty pounds per square inch, heating the compressed condenser to expel moisture and gases, again compressing the condenser, heating the condenser, impregnating the compressed condenser, cooling the condenser, and compressing the condenser under a relatively lower pressure during the cooling operation.

6. A method of manufacturing condensers which comprises preliminarily compressing a condenser under a pressure in the vicinity of sixty pounds per square inch, heating the compressed condenser to expel moisture and gases, again compressing the condenser, heating the condenser, impregnating the compressed condenser, cooling the condenser, compressing the condenser under a pressure in the vicinity of two pounds per square inch during a portion of the cooling operation, and gradually increasing this pressure.

7. A method of manufacturing condensers which comprises preliminarily compressing a condenser, heating the compressed condenser to expel moisture and gases, again compressing the condenser, heating the condenser, impregnating the compressed condenser, and compressing the condenser under an increasing pressure during cooling, the pressures for the preliminary and second pressures being higher than the final pressure applied to the impregnated condenser.

8. A method of manufacturing condensers which comprises preliminarily compressing a condenser under a pressure of at least of the order of sixty pounds per square inch, baking the condenser while compressed, again compressing the condenser under a pressure of at least of the order of sixty pounds per square inch, heating the condenser, subsequently impregnating the compressed condenser, cooling the condenser, and compressing the condenser during the cooling thereof to compensate for shrinkage.

9. A method of manufacturing condensers which comprises preliminarily compressing a condenser, drying the compressed condenser, again compressing the condenser, heating the condenser, then impregnating the compressed condenser and compressing the condenser after impregnation.

10. A method of manufacturing condensers which comprises preliminarily compressing a condenser, drying the compressed condenser, again compressing the condenser, heating the condenser, subsequently impregnating the compressed condenser, cooling the condenser, and compressing the condenser during the cooling thereof to compensate for shrinkage.

11. A method of manufacturing condensers which comprises preliminarily compressing a condenser, baking the compressed condenser, again compressing the condenser, heating the condenser, impregnating the compressed condenser, cooling the condenser, and compressing the condenser during the cooling thereof, the pressures of the preliminary and second compressions being higher than the final pressure.

12. A method of manufacturing condensers which comprises preliminarily compressing a condenser under a pressure in the vicinity of eighty pounds per square inch, drying the compressed condenser, again compressing the condenser, drying the condenser, then impregnating the compressed condenser and compressing the condenser after impregnation.

13. A method of manufacturing condensers which comprises preliminarily compressing a condenser in the vicinity of eighty pounds per square inch, heating the compressed condenser to dehydrate the same, again compressing the condenser under a pressure in the vicinity of eighty pounds per square inch, reheating the compressed condenser, subsequently impregnating the compressed condenser, and compressing the condenser after impregnation.

14. A method of manufacturing condensers which comprises preliminarily compressing a condenser, heating the compressed condenser to dehydrate the same while compressed, again compressing the condenser, reheating the condenser while compressed, impregnating the condenser while compressed at the residual pressure remaining from the second compression, cooling the condenser to a predetermined temperature without substantial pressure, and then compressing the condenser under an increase in pressure until the condenser is completely cooled.

5

15

20

35

40

50

60

65

WILLIAM B. WINES.